# EUROPEAN PATENT APPLICATION

(11) **EP 1 935 971 A1**
(43) Date of publication of application: **25.06.2008**
(21) Application number: 06126298.6
(22) Date of filing: 18.12.2006
(51) Int. Cl.: C11C 5/02, C11C 3/02

(54) **Partial acyl glyceride based biowaxes, biocandles prepared therfrom and their preparation methods**

(71) Applicant: Chant Oil Co., Ltd., Shu-Lin City Taipei Hsien (TW)
(72) Inventor: Lee, Yi-Fa, TAIPEI Hsien (TW)
(74) Representative: Collin, Jérôme

(57) **Abstract**

The present invention relates to a biowax comprising a partial acyl glyceride selected from the group consisting of a monoacylglyceride, a diacylglyceride and the combination thereof. The present invention also relates to a biocandle comprising a biowax and a wick, and to a method of producing the same.

## Description

### BACKGROUND OF THE INVENTION

### 1. Field of the Invention

The present invention relates to a biowax comprising partial acyl glycerides (PAG). The present invention also relates to biocandles formed from said biowax, and to a method for the production of the same.

### 2. Description of Related Arts

Many types of candles have already been developed on the market. Conventionally, candles are made by paraffin and/or natural waxes. Some typical candles prepared by conventional methods can be formed as container candles, votive candles, pillar candles, taper candles, tea-light candles and hurricane candles.

For a long time, it has been known that biowaxes, such as beeswax (myricyl palmitate) and spermaceti wax (cetyl palmitate), etc., can be used as natural waxes for the preparation of candles. Later, fossil waxes, such as paraffin, etc., are used as raw materials of candle waxes for the preparation of candles, in parallel with the development of the petroleum refining industry.

Today, paraffin-based waxes are major raw materials for the production of candles. The paraffin is produced from the residue left after refinement of fossil oils. It was found that paraffin can be completely burned, but it typically emits a smoke and produces an unpleasant odor when burning.

Palm stearin is a byproduct from palm oil refinery industry. The yield of palm stearin every year is huge and the price thereof is more inexpensive than paraffin. It has attempted to apply palm stearin as an ingredient of candle wax. However, due to the lower melting point property of the palm stearin, the compounding percentage in candle wax is limited and difficultly controlled. Even though the palm stearin may be hydrogenated to be one having a higher melting point, candles made therefrom are brittle and lack malleability. Thus, the application of palm stearin as an ingredient of candle wax is still limited.

To provide the candles having clean burning characteristics, extensive researches on candle waxes having low paraffin content have been conducted. For example, U.S Patent Nos. 6,503,285; 6,645,261; 6,770,104; 6,773,469; 6,797,020; and 5,824,572 disclose triacylglycerol based candle waxes, particularly those derived from various animal and/or plant sources, such as vegetable oil-source.

However, candle waxes formulated from vegetable oil-based materials often result in a variety of problems. It was found that vegetable oil-based candles have many disadvantages, such as cracking, air pocket formation and a natural product odor associated with soybean materials, as compared with paraffin-based candles. In addition, the soybean-based waxes have performance problems relating to optimum flame size, effective wax and wick performance matching for an even burn, maximum burning time, product color integration and/or product shelf life. Hence, to have the aesthetic and functional product surface and quality required by consumers, it is necessary to develop new substitutive vegetable oil-based waxes.

Accordingly, there exists a need to develop substitutive wax materials. Said substitutive wax materials have clean burning property when being used for forming candles. Preferably, such materials are biodegradable and derived from renewable raw materials. More preferably, the candle base wax materials have physical characteristics, such as melting point, hardness and/or malleability, etc., that permit the materials to be readily formed into candles having a pleasing appearance and/or feel to the touch, as well as having desirable olfactory properties.

Further, the Kyoto Protocol establishes the agreements of green issues in every aspect on the earth and its objective is "the stabilization of greenhouse gas concentrations in the atmosphere at a level that would prevent dangerous anthtopogenic interference with the climate system". As fossil fuel resources are scarce and the oil prices are soaring up, biomass fuels play a vital role on renewable energy supply chain. In the fast developing biodiesel supply chain, the oversupply of glycerol becomes an urgent problem to be solved.

### SUMMARY OF THE INVENTION

The present invention provides partial acyl glycerides (PAG)-based biowaxes. Such PAG-based biowax consumes majority of glycerol, thus ramify the biodiesel supply chain to solve the excess production of glycerol. In this invention, consuming the glycerol to produce PAG-based biowax and using the biowax in formation of green candle can facilitate the healthy developing of Carbon Cycle on Earth. Eventually it redirect the fossil energy to most valuable and feasible agricultural energy policy.

The present invention provides PAG-based biowax useful as candle wax. PAG-based biocandle has comparable burning characteristic with commercial candles made from paraffin wax in terms of flame length and is free of unpleasant odor. It has superior characteristics than paraffin wax which include low soot emission and high additives compatibility. It would be advantageous to use PAG-based biowax to replace paraffin wax.

In accordance with the present invention, the present invention further provides a biocandle comprising a biowax and a wick, wherein the biowax comprises partial acyl glycerides. Further, the candles may also be formed from PAG-based biowaxes containing paraffin and/or stearin as additional ingredients. The candles prepared therefrom exhibit uniform texture, translucent and fine grain crystalline structure. The candles are generally clean burning and emit very little soot Due to the combination of low soot emission and biodegradability, the production of candles from renewable raw materials makes the present candles a particularly environmentally friendly product.

In accordance with the present invention, it provides a method for preparing biocandles. With the method of the present invention, various types of biocandles, such as container candles, candle beads, etc. may be formed.

### BRIEF DESCRIPTION OF DRAWINGS

Figure 1 shows the gas chromatographic analysis result of GMP.
Figure 2 shows the gas chromatographic analysis result of partial acyl glycerids of Example 8 (defined as GMS_{IV=1.0}).
Figure 3 shows the gas chromatographic analysis result of partial acyl glycerides (defined as GMS_{IV=15}).
Figure 4 shows the gas chromatographic analysis result of partial acyl glycerides of Example 11 (defined as GMS_{IV=20})
Figure 5 shows the gas chromatographic analysis result of partial acyl glycerides of Example 12 (defined as GMS_{IV=30}).

### DETAILED DESCRIPTION OF THE INVENTION

According to the present invention, the biowax comprises partial acyl glycerides (PAG). Preferably, the biowax according to the present invention comprises about 20 wt.% to 100 wt.%, preferably 30 wt.% to 100 wt.%, of PAG, based on the total weight of the biowax.

As used herein, the term "biowax" refers to waxes produced from the raw materials derived from the biodiesel supply chain. As used herein, the term "partial acyl glyceride" refers to a glyceride selected from the group consisting of a monoacylglyceride (MAG), a diacylglyceride (DAG) and the combination thereof The partial acyl glyceride may be obtained by the esterification of glycerol molecules with one or two medium or long fatty acids chain. As used herein, the term "medium chain fatty acid" refers to a saturated or unsaturated fatty acid having 6 to 10 carbons, or a mixture thereof. Further, the term "long chain fatty acid" refers to a saturated or unsaturated fatty acid having 14 to 24 carbons, or a mixture thereof. More preferably, the acyl group has straight chains of C16, C18, C18:1, C18:2. According to the present invention, the partial acyl glyceride can be used alone, or in combination with triacyglycerides and/or other ingredients. The term "biocandle" used herein refers to candles produced from biowaxes.

According to the present invention, the biowax may further comprise triacylglyceride (TAG), stearin, or paraffin or a combination thereof as an additional ingredient. In one preferred embodiment of the present invention, the biowax comprises a monoacylglyceride (MAG), a diacylglyceride (DAG) and a triacylglyceride (TAG). The monoacylglyceride is used preferably in an amount of about 10 to 75 wt. %, more preferably in an amount of about 40 to 70 wt. %, based on the weight of the biowax. The diacylglyceride (DAG) is preferably used in amount of about 10 to 50 wt. %, more preferably in an amount of about 10 to 35 wt. %, based on the weight of the biowax. The triacylglyceride (TAG) is optionally used in an amount of about 5 to 50 wt. %, preferably in an amount of 10 to 40 wt. %, based on the weight of the biowax.

In the present invention, the biowax may optionally include minor amounts of other additives to modify the properties of the waxy materials. Examples of the additives incorporated into the biowax of the present invention include colorants, fragrances (e.g., fragrance oils), antioxidants, UV light absorber and migration inhibitors, and the like. Preferably, the biowax is blended with natural colorants to provide an even solid color distribution.

Biowax has a melting point of about 40 to 62°C. In one embodiment, the biowax has an Iodine Value of about 0.2 to 35.

In the present invention, the biowax can be formed into a desired shape. According to one preferred embodiment, the biowax may be formed into powdered or ground particles. Preferably, the biowax can be formed into beads by heating the biowax to a molten state and then spray cooling the molten biowax, or by means of a bead-manufacturing device commercially available from Chant Oil Co., Ltd. (Taiwan, R.O.C.). According to the present invention, the biowax may be shaped into beads having a diameter of about 0.5 to 1.2 mm.

In the present invention, the biowaxes are suitable as raw materials for the manufacture of biocandles.

According to the present invention, it provides a biocandle comprising a biowax and a wick, wherein the biowax comprises partial acyl glycerides (PAG). The biocandle is typically solid, firm but not brittle, generally somewhat malleable, with no free oil visible. In the present invention, the biocandles may be prepared by means of melt-processing to form the desired shape of candles, such as pillar candles, tea light candles, etc.

In the present invention, in order to fully benefit from the environmentally-safe aspect of said PAG-based biowax, it is desirable to use a wick which does not have a metal core, such as a lead or zinc core. One example of a suitable wick material is a braided cotton wick. The wick may apply standard wicks employed with other waxes (e.g., paraffin and/or beeswax).

According to the present invention, it further provides a method of preparing a biocandle, comprises the steps of: 1) heating the PAG-based biowax to a molten state, 2) introducing the molten biowax into a mold, wherein the mold includes a wick disposed therein, 3) cooling the molten biowax in the mold, and 4) solidifying the biowax, and then removing the solidified biowax from the mold.

The present invention further provides a method for preparing a biocandle comprising heating the PAG-based biowax to a molten state, spray cooling the biowax to form 0.5 to 1.2 mm beads and compressing the biowax beads into a mold to form as candles.

For preparation of biocandles, it is important that the colorants, if present, need be dissolved in the PAG-based biowax in order to prevent insoluble particles from blocking the biowax flow in the wick. Generally, the blocked biowax flow results in a poor candle bum. Further, the color of the biowax may also affect the dying performance. Most fragrances can be applied to the biowax to improve the performance of the resulting biocandles, such as stability, reactivity, color, etc.

According to the present invention, the resulting biocandles are clean burning and emit very little soot.

In the present invention, all numbers expressing quantities of ingredients, properties, etc. in the specification and claims are to be understood as being modified in all instances by the term "about", and all parts and percentages referred to in this specification and claims are by weight, unless otherwise specified.

The invention is illustrated in greater detail by the examples described below. The examples are not intended in any way to limit the scope of the invention. Notwithstanding that the numerical ranges and parameters setting forth the broad scope are approximations, the numerical values set forth in the specific example are reported as precisely as possible. Any numerical value, however, inherently contains certain errors necessarily resulting from the standard deviation found in its respective testing measurements.

### Examples

### A. Gas Chromatographic Analysis of PAG

GC Model: YOUNGLIN ACME 6000M GC
GC Conditions:
   1. Column: QUADREX fused silica capillary column; 007-65HT-25W-0.1F, 0.32mmID
   2. Detector: FID
   3. Carrier Gas: Nitrogen
   4. Oven Temperature:
      1) 80°C (Hold 1 min), and to 240°C in a rate of 20°C/min;
      2) 240°C, and to 360°C in a rate of 4°C/min;
      3) 360°C (Hold 11 min)
   5. Injector Temperature: 280°C
   6. Detector Temperature: 360°C
   7. Determination Range: 6x10³mV
Preparation of Samples:
   Homogeneously mixing 0.2 gm of sample with 5cc chloroform.
Analysis Conditions:
   1. Sample Content: 0.2 µl
   2. Analysis Time: 50 mins

### B. Components for the Preparation of waxes

Component 1: Paraffin wax, supplied by Taiwan Wax Co., Ltd., has the physical properties listed on Table 1.

**Table 1**

| Physical Property | Test Method | Value |
|---|---|---|
| M.P., °C | ASTM D87 | 59.8 |
| Needle Penetration at 25°C, mm | ASTM D 1321 | 15.5 |
| Kinetic Viscosity at 100°C, cps | ASTM D445 | 4.382 |
| Oil Content, wt.% | ASTM D721 | 0.116 |
| Color | ASTM D156 | 30 |
| Carbon Distribution | ASTM D5442 | C₂₀ ~ C₄₆ |
| <C₂₆ | | 16.48% |
| C₂₆₋₂₉ | | 23.78% |
| C₂₉₋₃₂ | | 23.05% |
| C₃₂₋₄₄ | | 36.69% |
| >C₄₄ | | nil |
| n-Paraffin | | 51.05% |

Component 2: Fatty acid S1801, supplied by P.T. MUSIM MAS., has the physical properties listed on Table 2.

**Table 2**

| Physical Property | Test Method | Value |
|---|---|---|
| Acid Value, mg KOH/g | ASTM D 1980-87 | 210.2 |
| Saponification Value, mg KOH/g | ASTMD1962-85 | 211.4 |
| Iodine Value, g Iodine/100g | ASTM D 1959-97 | 0.13 |
| M.P., °C | ASTM D 1982-85 | 55.4 |
| Fatty Acid Carbon Chain Composition, % | ASTM D 1983-90 | |
| C12+14 | | 0.4 |
| C16 | | 57.67 |
| C18 | | 41.3 |
| Others | | 0.5 |

Component 3: Fatty acid 1698, supplied by P.T. MUSIM MAS., has the physical properties listed on Table 3.

**Table 3**

| Physical Property | Value |
|---|---|
| Acid Value, mg KOH/g | 218.5 |
| Saponification Value, mg KOH/g | 220 |
| Iodine Value, g Iodine/100g | 0.1 |
| M.P., °C | 62.0 |
| Fatty Acid Carbon Chain Composition, % | |
| C12+14 | 0.3 |
| C16 | 98.6 |
| C18 | 1.1 |
| Others | 0.5 |

Component 4: Two types of RBD Palm Stearin supplied by P.T. MUSIM MAS. having the physical properties listed Table 4.

**Table 4**

| Physical Property | Type 1 | Type 2 |
|---|---|---|
| Free Fatty Acid, % | 0.057 | 0.01 |
| Iodine Value, g Iodine/ 1 00g | 20.4 | 33.3 |
| M.P., °C | 56.5 | 51 |
| Fatty Acid Carbon Chain Composition, % | | |
| C16 | 72.00 | 59.8 |
| C18 | 5.10 | 3.67 |
| C18:1 | 16.22 | 29.7 |
| C18:2 | 3.67 | 5.22 |

Component 5: Hardened Fat FO81, made by hydrogenation of RBD palm stearin (Type 2, Component 4) at a temperature of from 170 to 200°C and at a pressure of 3kg in the presence of Ni catalyst (0.2%) for 4 hours, has the physical properties listed on Table 5.

**Table 5**

| Physical Property | Value |
|---|---|
| Acid Value, mg KOH/g | 1.2 |
| Saponification Value, mg KOH/g | 196.8 |
| Iodine Value, g Iodine/100g | 0.4 |
| M.P., °C | 57 |
| Color Gardner | 1.3 |
| Fatty Acid Carbon Chain Composition, % | |
| C16 | 59.8 |
| C18 | 35.6 |

Component 6: Partial Acyl Glyceride defined as GMP, made by the reaction of 200 gm of Fatty Acid 1698 (Component 3) with 72 gm of glycerol at 250 °C for 5 hours, has the physical properties listed on Table 6a and GC analysis result and data respectively shown in Figure 1 and Table 6b.

**Table 6a**

| Physical Property | Value |
|---|---|
| Free Fatty Acid, % | 1.2 |
| M.P., °C | 56 |
| MAG % | 64.0 |
| DAG, % | 25.5 |
| TAG, % | 9.3 |

| | |
|---|---|
| MAG: Monoacylglyceride DAG: Diacylglyceride TAG: Triacylglyceride | |

**Table 6b**

| Peak No. | Component | Retention Time (second) | Area | Percentage (%) |
|---|---|---|---|---|
| 1 | FFA | 8.813 | 146.88 | 1.20 |
| 2 | GMP | 14.424 | 7845.39 | 63.98 |
| 3 | GDP | 31.754 | 3132.86 | 25.54 |
| 4 | GTP | 48.118 | 1137.85 | 9.28 |

| | | | | |
|---|---|---|---|---|
| FFA: Free Fatty Acid GMP: Glycerol Monopalmitate GDP: Glycerol Dipalmitate GTP: Glycerol Tripalmitate | | | | |

Component 7: Partial Acyl Glyceride defined as GMS_{IV=1.0,} made by the reaction of 200 gm of Fatty Acid S1801 (Component 2) with 72 gm of glycerol at 250 °C for 5 hours, has the physical properties listed on Table 7a and GC analysis result and data respectively shown in Figure 2 and Table 7b.

**Table 7a**

| Physical Property | Value |
|---|---|
| Acid Value, mg KOH/g | 0.4 |
| Iodine Value, mg KOH/g | 0.2 |
| Color, APHA | 140 |
| M.P., °C | 56 |
| MAG, % | 62.6 |
| DAG, % | 28.8 |
| TAG, % | 7.6 |

**Table 7b**

| Peak No. | Component | Retention Time (second) | Area | Percentage (%) |
|---|---|---|---|---|
| 1 | G | 3.539 | 519.91 | 0.65 |
| 2 | FFA | 6.525 | 233.16 | 0.29 |
| 3 | FFA | 7.350 | 46.61 | 0.06 |
| 4 | Mono-Glyceride | 10.453 | 48623.36 | 60.90 |
| 5 | Di-Glyceride | 16.861 | 215.56 | 0.27 |
| 6 | Di-glyceride | 23.320 | 24237.86 | 30.36 |
| 7 | Tri-Glyceride | 36.047 | 5964.83 | 7.47 |

| | | | | |
|---|---|---|---|---|
| G: Glycerol | | | | |

Component 8: Partial Acyl Glyceride defined as GMS_{IV=15}, made by a 200gm of mixture of equal amount of FO81 (Component 5) and RBD palm stearin (Type 2, Component 4) with 40 gm of glycerol at 250 °C for 8 hours, has the physical properties listed on Table 8a and GC analysis result and data respectively shown in Figure 3 and Table 8b.

**Table 8a**

| Physical Property | Value |
|---|---|
| M.P., °C | 46 |
| MAG, % | 68.35 |
| DAG, % | 15.69 |
| TAG, % | 11.72 |

**Table 8b**

| Peak No. | Component | Retention Time (second) | Area | Percentage (%) |
|---|---|---|---|---|
| 1 | G | 2.572 | 83.89 | 0.62 |
| 2 | FFA | 6.424 | 487.76 | 3.6 |
| 3 | FFA | 7.287 | 558.61 | 4.14 |
| 4 | Mono-Glyceride | 9.360 | 8665.79 | 64.21 |
| 5 | Di-Glyceride | 15.445 | 10.99 | 0.08 |
| 6 | Di-glyceride | 19.710 | 2106.60 | 15.61 |
| 7 | Tri-Glyceride | 27.898 | 6.40 | 0.05 |
| 8 | Tri-Glyceride | 29.627 | 42.31 | 0.31 |
| 9 | Tri-Glyceide | 31.626 | 1532.99 | 11.36 |

Component 9: Partial Acyl Glyceride defined as GMS_{IV=20}, made by the reaction of 200 gm of RBD palm stearin (Type 1, Component 4) with 40 gm of glycerol at 250 °C for 8 hours, has the physical properties listed on Table 9a and GC analysis result and data respectively shown in Figure 4 and Table 9b.

**Table 9a**

| Physical Property | Value |
|---|---|
| Color | 1.4 |
| M.P., °C | 46 |
| MAG % | 49.6 |
| DAG,% | 11.1 |
| TAG, % | 33.1 |

**Table 9b**

| Peak No. | Component | Retention Time (second) | Area | Percentage (%) |
|---|---|---|---|---|
| 1 | FFA | 6.499 | 989.15 | 5.25 |
| 2 | Mono-Glyceride | 9.405 | 8776.13 | 46.60 |
| 3 | Di-Glyceride | 19.948 | 2471.18 | 13.12 |
| 4 | Tri-Glyceride | 27.846 | 16.10 | 0.09 |
| 5 | Tri-Glyceride | 32.31 | 6582.08 | 34.95 |

Component 10: Partial Acyl Glyceride designed as GMS_{IV=30}, made by the reaction of 200 gm of RBD palm stearin (Type 2, from Component 4) with 40 gm of glycerol at 250 °C for 8 hours, has the physical properties listed on Table 10a and GC analysis result and data respectively shown in Figure 5 and Table 10b.

**Table 10a**

| Physical Property | Value |
|---|---|
| M.P., °C | 42 |
| MAG,% | 66.2 |
| DAG, % | 13.4 |
| TAG, % | 13.3 |

**Table 10b**

| Peak No. | Component | Retention Time (second) | Area | Percentage (%) |
|---|---|---|---|---|
| 1 | G | 2.489 | 49.89 | 0.18 |
| 2 | FFA | 6.511 | 1933.86 | 6.93 |
| 3 | Mono-Glyceride | 9.507 | 18463.30 | 66.20 |
| 4 | Di-Glyceride | 13.502 | 14.22 | 0.05 |
| 5 | Di-Glyceride | 15.504 | 20.38 | 0.07 |
| 6 | Di-Glyceride | 20.023 | 3715.59 | 13.32 |
| 7 | Tri-Glyceride | 27.924 | 18.28 | 0.07 |
| 8 | Tri-glyceride | 33.699 | 3674.74 | 13.18 |

### C. Preparation of container candle (as listed in Table 11) to be tested:

Various components were mixed in an equal weight amount and molten. The molten waxes were poured into an aluminum cup having 15mm height x 37.5mm diameter with a 23mm length of braided cotton wick disposed in the middle of the cup. The resulting candles were cooled and solidified for the burning test.

### Examples 1 to 13

The container candles were prepared according to the components and contents listed on Table 11.

### D. Burning Test

The burning performances of biocandles prepared from partial acyl glyceride (PAG) based biowaxes were curried out by folloing the steps below:
1. numbering and weighing each of container candles having various amounts of components;
2. placing the container candle separated by a distance of 100 mm on the experimental table;
3. placing a plaster slab 75 mm above the table, to observe the smoke emiting from the candles, when burning;
4. igniting the container candles and starting timing; measuring the flame heights of each container candles as soon as possible, when the wax is molten around each of the wick (about 5-6 minutes);
5. measuring the flame heights at an interval of one hour;
6. measuring the temperatures at the highest point of inside flame for each container candle after 60 minutes;
7. weighing each container candle after one of them burned out; and then calculating its burning rates of each container candle.

The burning test results of the container candles are shown on Table 11.

**Table 11**

| Example No. | 1 | 2 | 3 | 4 | 5 | 6 | 7 | 8 | 9_{{Comparative}} | 10 | 11 | 12 | 13 |
|---|---|---|---|---|---|---|---|---|---|---|---|---|---|
| Component 1: Paraffin wax (weight, g) | 3.91 | 4.94 | 5.23 | | | | 7.78 | | 7.49 | | | | |
| Component 2: S1801 (weight, g) | 3.91 | 4.94 | | 5.49 | 7.99 | | | | 7.49 | | | | |
| Component 5: FO81 (weight, g) | 3.91 | | 5.23 | 5.49 | | 7.78 | | | | | | | |
| Component 6: GMP (weight, g) | | | | | | | | | | | | | 21.59 |
| Component 7: GMS_{IV=1.0} (weight, g) | 3.91 | 4.94 | 5.23 | 5.49 | 7.99 | 7.78 | 7.78 | 15.32 | | | | | |
| Component 8: GMS_{IV=15} (weight, g) | | | | | | | | | | 23.26 | | | |
| Component 9: GMS_{IV=20} (weight, g) | | | | | | | | | | | 22.87 | | |
| Component 10: GMS_{IV=30}(weight, g) | | | | | | | | | | | | 22.04 | |

| Properties | | | | | | | | | | | | | |
|---|---|---|---|---|---|---|---|---|---|---|---|---|---|
| MP(°C) | 50.5 | 52 | 52 | 51.5 | 52 | 53 | 57.5 | 54 | 52 | 46 | 46 | 42 | 52 |
| Initial weight (g) | 15.64 | 14.82 | 15.69 | 16.47 | 15.98 | 15.56 | 15.56 | 15.32 | 14.98 | 23.26 | 22.87 | 22.04 | 21.59 |
| Remain weight (g), after 132 min. | 4.77 | 3.10 | 3.64 | 6.76 | 7.37 | 5.60 | 2.78 | 3.62 | 3.88 | 14.24 | 14.00 | 15.11 | 10.60 |
| Bum rate (g/hr) | 4.94 | 5.32 | 5.48 | 4.42 | 3.91 | 4.53 | 5.80 | 5.32 | 5.04 | 4.10 | 4.03 | 3.15 | 5.00 |
| Flame Temperature (°C) | 731 | 768 | 757 | 711 | 729 | 777 | 839 | 881 | 806 | 835 | 740 | 668 | 820 |
| Flame Height (mm), after 6 min. | 26 | 27 | 25 | 23 | 24 | 24 | 27 | 22 | 33 | 15 | 25 | 20 | 25 |
| Flame Height (mm), after 70 min. | 26 | 26 | 26 | 22 | 15 | 25 | 30 | 22 | 28 | 18 | 18 | 10 | 18 |
| Flame Height (mm), after 132 min. | 21 | 24 | 30 | 20 | 15 | 23 | 23 | 21 | 27 | 15 | 17 | 6 | 24 |

As shown on Table 11, the biocandles made by the biowaxes of the present invention, together with a balanced amount of paraffin and/or stearin, exhibit excellent wax flow through wicks by visual appearance. Meanwhile, the biocandles of the present invention show steady burn rate and good appearances, such as color, fragrance and clarity, and also emit low soot when burning and good smell.

While the embodiments of the present invention described herein are presently preferred, various modifications and improvements can be made without departing from the spirit and scope of the present invention. The scope of the present invention is indicated by the appended claims, and all changes that fall within the meaning and range of equivalents are intended to be embraced therein.

## Claims

1. A biowax, comprising a partial acyl glyceride selected from the group consisting of monoacylglycerides and diacylglycerides, and the combination thereof.

2. The biowax of claim 1, wherein the partial acyl glyceride is present in an amount of 20 wt.% to 100 wt.%, based on the total weight of the biowax.

3. The biowax of claim 1, wherein the partial acyl glyceride is present in an amount of 30 wt.% to 100 wt.%, based on the total weight of the biowax.

4. The biowax of claim 1, further comprising triacylglycerides.

5. The biowax of claim 4, wherein the monoacylglycerides are in an amount of about 10 to 75 wt. % and the diacylgiycerides are in an amount of about 10 to 50 wt. %, and the triacylglycerides are in an amount of about 5 to 50 wt. %, based on the weight of the biowax.

6. The biowax of claim 5, wherein the triacylglycerides are in an amount of about 10 to 40 wt. %, based on the weight of the mixture.

7. The biowax of any one of claim 1 to 6, which further comprises a colorant, antioxidant or fragrance oil.

8. The biowax of claim 7, which is formed into beads having a diameter of about 0.5 to 1.2 mm.

9. The biowax of any one of claims 1 to 6, which has a melting point of about 40 to 62°C .

10. The biowax of any one of claims 1 to 6, which has an Iodine Value of about 0.2 to 35.

11. A biocandle comprising a biowax according to any one of claims 1 to 6 and a wick.

12. A method of producing a biocandle, comprising the steps of:
1) heating the PAG-based biowax to a molten state;
2) introducing the molten biowax into a mold, wherein the mold includes a wick disposed therein;
3) cooling the molten biowax in the mold; and
4) solidifying the biowax, and then removing the solidified biowax from the mold;
wherein the biowax comprises a partial acyl glyceride selected from the group consisting of monoacylglycerides, diacylglycerides and the combination thereof.

13. A method of producing a biocandle, comprising the steps of
1) heating the PAG-based biowax to a molten state;
2) spray cooling the molten biowan to form 0.5 to 1.2 mm beads; and
3) compressing the biowax beads into a mold to form as candles.
